

## UNITED STATES PATENT OFFICE.

HERBERT W. GEPP, OF MELBOURNE, VICTORIA, AUSTRALIA, ASSIGNOR TO ELECTROLYTIC ZINC COMPANY OF AUSTRALASIA PROPRIETARY LIMITED, OF MELBOURNE, AUSTRALIA.

## ROASTING OF ZINC SULPHIDE ORES PREPARATORY TO LEACHING.

No Drawing.

Application filed September 5, 1919. Serial No. 321,949.

To all whom it may concern:

Be it known that I, HERBERT WILLIAM GEPP, general manager of Electrolytic Zinc Company of Australasia Proprietary Limited, residing at Collins House, 360-366 Collins Street, Melbourne, in the State of Victoria, Commonwealth of Australia, a subject of the King of Great Britain, have invented certain new and useful Improvements in the 5 Roasting of Zinc Sulphide Ores Preparatory to Leaching, of which the following is a specification.

This invention relates to certain improvements in the roasting of sulphide ores preparatory to leaching and refers more especially to the roasting of zinc blende preparatory to leaching with sulphuric acid or spent electrolyte for the formation of zinc sulphate solution prior to electrolysis for the deposition of metallic zinc or spelter.

The invention is applicable to any process which involves the preparation of solutions of zinc sulphate such as the manufacture of "lithopone" and such like processes.

This invention relates to the treatment of concentrates, slimes, tailings and other metallurgical products as well as to crude ores and it will be understood that in this specification the term "ores" will include metalliferous products as well as the crude material.

The methods which have become standard for the roasting of zinc sulphide ores for the distillation process have been found to be more or less unsatisfactory when the roasted ore is to be leached with sulphuric acid.

In the roasting of ores preparatory to distillation it is sought to eliminate the sulphur whether present as sulphide or sulphate.

On the other hand when the ores are to be leached with sulphuric acid the presence of sulphates is not a disadvantage; in fact it may even be an advantage in cases where a steady consumption of sulphuric acid has to be met in the subsequent leaching. This of course, is true more or less in the electrolytic process, and still more so in the manufacture of lithopone where practically the whole of the sulphuric acid appears in the final product as barium sulphate.

In the electrolytic zinc process it is usually necessary to add a quantity of sulphuric acid

to the leaching solution in order to make up losses occasioned in the working of the process and to maintain the proper concentration of zinc in the solution.

In the roasting of zinc sulphide ores when it is desired to effect the more or less complete elimination of the sulphur and to obtain a "dead" roast or "sweet" roast (such as is the practice preparatory to the distillation process) it has been found necessary to maintain the operation at a high temperature and if the gases are to be used for the manufacture of sulphuric acid the admission of air must be carefully controlled.

In the roasting of zinc sulphide ores when it is desired to effect a "sulphating" roast and to obtain a maximum proportion of metallic sulphates it is necessary to maintain the temperature as low as possible to prevent the breaking up of the metallic sulphates formed (and in particular zinc sulphate) and further an excess of air is required to effect the oxidation to sulphates which renders the gases too dilute for the manufacture of sulphuric acid.

The object of this invention is to provide certain improvements in the roasting of zinc sulphide ores preparatory to leaching whereby a "sulphating" roast is effected with the formation of a maximum quantity of metallic sulphates which are introduced into the leaching solution thereby reducing the amount of sulphuric acid which would otherwise be required to be added to the leaching solutions or avoiding such additions altogether.

I accomplish this object by conducting the roasting operation under such conditions that a maximum of metallic sulphates are formed. This is preferably effected by conducting the roasting operation in two stages. The first stage is carried out under such conditions as obtain with an ordinary roast that is to say with the maintenance of a relatively high temperature and with a carefully controlled supply of air to ensure a sufficient concentration of  $\text{SO}_2$  for the manufacture of sulphuric acid, the sulphur contents being reduced to such an amount as may be necessary for the subsequent operation. The second stage is effected at a relatively lower temperature and under such conditions of

air supply and amount of available sulphur present as is calculated to give a maximum yield of metallic sulphates.

This two-stage roasting operation may be conducted in either of two ways that is either by conducting the first operation for a partial elimination of the sulphur, and the second operation for the formation of a maximum amount of sulphates or alternatively by conducting the first operation for the more or less complete elimination of the sulphur and then adding "green" or unroasted sulphides and roasting under such conditions that a maximum amount of sulphates is formed.

I have discovered that the efficiency of the sulphate formation increases as the sulphide sulphur contents decrease. For example in the roasting of an ore containing 28% sulphur at a temperature suitable for the formation of sulphates it has been found that with the reduction of the sulphur down to 8% only the lead was sulphated but that when the reduction was continued it was possible to secure a 40% conversion to sulphate of the remaining 8 units of sulphur. It was further found that if the reduction of the sulphur in the first instance had been carried down to 6% it was possible to obtain 50% conversion to sulphate of those remaining 6 units. It has been found that the conversion of the last unit of sulphide sulphur to sulphate is almost quantitative.

In proceeding as indicated in the former alternative—that is to say when conducting the first operation for a partial elimination of the sulphur) the preliminary roasting is conducted in the same manner as heretofore, being effected in a suitable furnace at a relatively high temperature with regulation of air supply so that the gases are suitable for the formation of sulphuric acid. In this preliminary roasting operation the sulphur contents are reduced to approximately from 6 to 10%. In the second operation the roasting is carried forward with a view to converting a maximum amount of sulphur to sulphate sulphur which is attained by definite control over both temperature and draught and with the addition where necessary at certain stages of further sulphur such as by adding green or unroasted sulphides. The temperature in the second operation is maintained at a range of 650° C. to 750 C. being preferably at 725° C. at which temperature rapid roasting is effected and overheating of the charge avoided. Furthermore, during this second operation it is necessary to provide such conditions that a sufficient excess of air and a sufficient proportion of  $\text{SO}_2$  is present in the furnace and that the proportion of carbon dioxide is maintained as low as possible.

In carrying out this second operation the ore after the preliminary roast may be

mixed with a proportion of material which has already been submitted to a sulphating roast. For example I have found that in treating a material in which the sulphur contents had been reduced to 60% as sulphide, four parts of the same were mixed with one part of material which has already been roasted to sulphate whereby the said mixture contained approximately 4.8% sulphide sulphur and 2.2% sulphate sulphur. In this case a final product was obtained containing 5% sulphur present as sulphate.

The second alternative is adopted where the roasted calcine is delivered to the reduction works with the sulphide sulphur reduced to a minimum and also for the treatment of oxidized ores.

In this case it is necessary to add sulphide sulphur preferably in the form of green or unroasted concentrates during the sulphating operation. As the efficiency of the sulphate formation increases as the percentage of sulphide sulphur decreases it is preferable to add the green concentrates successively so regulating the additions that the percentage of sulphide sulphur in the charge does not rise above 2%.

In the experiments which have been conducted by me the ores operated on all contained about 15% of iron as oxides and it would appear that this functions as a catalyst converting the sulphur dioxide in the presence of excess of air into the trioxide which is then absorbed by the zinc oxide to form the sulphate.

This type of roasting leads to the diminution of the amount of ferrite formed directly owing to the lower temperature, and indirectly owing to the decomposition of the ferrite formed during the earlier stages of the roast by sulphuric anhydride formed during the latter stages.

By these means it is possible to obtain such a degree of sulphating as may be required for the purpose of introducing into the leaching liquor sufficient sulphuric acid as sulphates to make up for losses or for withdrawals from the solutions for other purposes (such as the making of lithopone).

Furthermore a subsequent roasting or heating of calcines immediately precedent to the leaching may serve other useful purposes. In some cases especially where it is necessary to transport the roasted calcine from one place to another for treatment, it is customary to wet down the material to prevent dusting during handling. In this and other ways chlorine is introduced which has been found prejudicial to the electrolytic process and it has been found that a final roast as above described has the effect of volatilizing the chlorides and thereby eliminating the same and at the same time converting any remaining ferrous iron to ferric iron.

70

80

85

90

95

100

105

110

115

120

125

130

I claim:—

1. A process for treating zinc sulphide ores which comprises first bringing the sulphide sulphur contents thereof to a value of about 6% to 10% of the weight of the ore by any suitable means and then roasting the ore at a relatively low temperature in the presence of air and so controlling the supply of air that the formation of a maximum amount of metallic sulphates is effected. 5
2. A process for the roasting of zinc sulphide ores in which the sulphur contents are first reduced to from 6 to 10% (approximately) then diluting the sulphide sulphur contents by mixing the same with a proportion of ore relatively free from sulphide sulphur and then roasting at a relatively low temperature in the presence of an excess of air under such conditions that the formation 10 of a maximum amount of metallic sulphates is effected. 20
3. A process for the roasting of zinc sulphide ores in which the sulphur contents are first reduced to from 6 to 10% approximately then diluting the sulphide sulphur 25

contents by the addition of ore which has previously been subjected to a sulphating operation and then roasting the mixture at a relatively low temperature in the presence of an excess of air under such conditions 30 that the formation of a maximum amount of metallic sulphates is effected.

4. In the roasting of zinc sulphide ores as hereinbefore described in which the sulphide sulphur contents are reduced to a 35 relatively low percentage and then roasted at a relatively low temperature in presence of excess of air the addition of a catalyst (such as ferric oxide) for the purpose of promoting the conversion of sulphur dioxide to sulphur trioxide for the formation of a maximum amount of metallic sulphates substantially as described. 40

In testimony whereof I have signed my name to this specification in the presence of 45 two subscribing witnesses.

HERBERT W. GEPP.

Witnesses:

CLEM A. HACK,  
G. CULLEN.